



US006132913A

# United States Patent [19]

Fuller et al.

[11] Patent Number: 6,132,913

[45] Date of Patent: Oct. 17, 2000

[54] **PHOTORECEPTOR OVERCOATINGS  
CONTAINING HYDROXY  
FUNCTIONALIZED AROMATIC DIAMINE,  
HYDROXY FUNCTIONALIZED  
TRIARYLAMINE AND CROSSLINKED  
ACRYLATED POLYAMIDE**

[75] Inventors: **Timothy J. Fuller**, Pittsford; **John F. Yanus**, Webster; **Damodar M. Pai**, Fairport; **William W. Limburg**, Penfield; **Markus R. Silvestri**, Fairport; **Dale S. Renfer**; **Anthony T. Ward**, both of Webster; **Paul J. DeFeo**, Sodus Point; **Harold F. Hammond**, Webster; **Robert W. Nolley**, Rochester, all of N.Y.

[73] Assignee: **Xerox Corporation**, Stamford, Conn.

[21] Appl. No.: **09/265,187**

[22] Filed: **Mar. 9, 1999**

## Related U.S. Application Data

[62] Division of application No. 09/182,375, Oct. 29, 1998, Pat. No. 5,976,744.

[51] **Int. Cl.<sup>7</sup>** ..... **G03G 5/47**; G03G 13/22

[52] **U.S. Cl.** ..... **430/59**; 430/60; 430/66; 430/67; 430/126; 252/500; 528/310

[58] **Field of Search** ..... 528/310; 430/59, 430/60, 66, 67, 126; 252/500

## [56] References Cited

### U.S. PATENT DOCUMENTS

|           |         |                |       |         |
|-----------|---------|----------------|-------|---------|
| 4,871,634 | 10/1989 | Limburg et al. | ..... | 430/54  |
| 5,368,967 | 11/1994 | Schank et al.  | ..... | 430/59  |
| 5,612,157 | 3/1997  | Yuh et al.     | ..... | 430/58  |
| 5,670,291 | 9/1997  | Ward et al.    | ..... | 430/152 |
| 5,681,679 | 10/1997 | Schank et al.  | ..... | 430/59  |
| 5,702,854 | 12/1997 | Schank et al.  | ..... | 430/59  |
| 5,709,974 | 1/1998  | Yuh et al.     | ..... | 430/59  |
| 5,976,744 | 11/1999 | Fuller et al.  | ..... | 430/59  |

*Primary Examiner*—P. Hampton-Hightower

## [57] ABSTRACT

A crosslinkable coating composition including an alcohol soluble acrylated polyamide containing alkoxyethyl or alkoxyalkylmethyl groups attached to amide nitrogen atoms, a crosslinking catalyst and a mixture of a hydroxy functionalized aromatic diamine with a hydroxy functionalized triarylamine. A coating is formed from this composition.

**14 Claims, No Drawings**

**PHOTORECEPTOR OVERCOATINGS  
CONTAINING HYDROXY  
FUNCTIONALIZED AROMATIC DIAMINE,  
HYDROXY FUNCTIONALIZED  
TRIARYLAMINE AND CROSSLINKED  
ACRYLATED POLYAMIDE**

This application is a divisional of application Ser. No. 09/182,375, filed Oct. 29, 1998 now U.S. Pat. No. 5,976, 744.

**BACKGROUND OF THE INVENTION**

This invention relates in general to coating compositions and, more specifically, to compositions and coated electro-photographic imaging members comprising a hydroxy functionalized aromatic diamine, a hydroxy functionalized triarylamine and a crosslinked acrylated-polyamide.

Electrophotographic imaging members, i.e., photoreceptors, typically comprise at least one photoconductive layer formed on an electrically conductive substrate. The photoconductive layer is a good insulator in the dark so that electric charges are retained on its surface. Upon exposure to light, the charge is dissipated.

An electrostatic latent image is formed on the photoreceptor by first uniformly depositing an electric charge over the surface of the photoconductive layer by one of any suitable means well known in the art. The photoconductive layer functions as a charge storage capacitor with charge on its free surface and an equal charge of opposite polarity (the counter charge) on the conductive substrate. A light image is then projected onto the photoconductive layer. On those portions of the photoconductive layer that are exposed to light, the electric charge is conducted through the layer reducing the surface charge. The portions of the surface of the photoconductive not exposed to light retain their surface charge. The quantity of electric charge at any particular area of the photoconductive surface is inversely related to the illumination incident thereon, thus forming an electrostatic latent image. After development of the latent image with toner particles to form a toner image, the toner image is usually transferred to a receiving member such as paper. Transfer is effected by various means such as by electrostatic transfer during which an electrostatic charge is applied to the back side of the receiving member while the front side of the member is in contact with the toner image.

The photodischarge of the photoconductive layer requires that the layer photogenerate free charge carriers and transport this charge through the layer thereby neutralizing the charge on the surface. Two types of photoreceptor structures have been employed. One type comprises multilayer structures wherein separate layers perform the functions of charge generation and charge transport, respectively, and single layer photoconductors which perform both functions. These layers are formed on an electrically conductive substrate and may include an optional charge blocking and an adhesive layer between the conductive layer and the photoconducting layer or layers. Additionally, the substrate may comprise a non-conducting mechanical support with a conductive surface. Other layers for providing special functions such as incoherent reflection of laser light, dot patterns for pictorial imaging or subbing layers to provide chemical settings and/or a smooth coating surface may optionally be employed.

One common type of photoreceptor is a multilayered device that comprises a conductive layer, a blocking layer, an adhesive layer, a charge generating layer, and a charge

transport layer. The charge transport layer can contain an active aromatic diamine molecule, which enables charge transport, dissolved or molecularly dispersed in a film forming binder. This type of charge transport layer is described, 5 for example in U.S. Pat. No. 4,265,990. Other charge transport molecules disclosed in the prior art include a variety of electron donors, aromatic amines, oxadiazoles, oxazoles, hydrazones and stilbenes for hole transport and electron acceptor molecules for electron transport. Another type of charge transport layer has been developed which utilizes a charge transporting polymer wherein the charge transporting moiety is incorporated in the polymer as a group pendant from the polymer backbone or as a moiety in the backbone of the polymer. These types of charge transport polymers include materials such as poly(N-vinylcarbazole), polysilylenes, and others including those described, for 10 example, in U.S. Pat. Nos. 4,618,551, 4,806,443, 4,806,444, 4,818,650, 4,935,487, and 4,956,440. The disclosures of these patents are incorporated herein in their entirety.

Charge generator layers comprise amorphous films of selenium and alloys of selenium and arsenic, tellurium, germanium and the like, hydrogenated amorphous silicon and compounds of silicon and germanium, carbon, oxygen, nitrogen, and the like, fabricated by vacuum evaporation or 15 deposition. The charge generator layers may also comprise inorganic pigments of crystalline selenium and its alloys; Group II-VI compounds; and organic pigments such as quinacridones, polycyclic pigments such as dibromo anthanthrone pigments, perylene and perinone diamines, 20 polynuclear aromatic quinones, azo pigments including bis-, tris- and tetrakis-azos; and the like, dispersed in a film forming polymeric binder and fabricated by solvent coating techniques.

Phthalocyanines have been employed as photogenerating 25 materials for use in laser printers utilizing infrared exposure systems. Infrared sensitivity is required for photoreceptors exposed to low cost semiconductor laser diode light exposure devices. The absorption spectrum and photosensitivity of the phthalocyanines depend on the central metal atom of the compound. Many metal phthalocyanines have been 30 reported and include, oxyvanadium phthalocyanine, chloro-aluminum phthalocyanine, copper phthalocyanine, oxytitanium phthalocyanine, chlorogallium phthalocyanine, magnesium phthalocyanine and metal-free phthalocyanine. The 35 phthalocyanines exist in many crystal forms which have a strong influence on photogeneration.

One design criteria for the selection of the photosensitive pigment for a charge generator layer and the charge transporting molecule for a transport layer is that, when light 40 photons photogenerate holes in the pigment, the holes must be efficiently injected into the charge transporting molecule in the transport layer. More specifically, the injection efficiency from the pigment to the transport layer should be high. A second design criterion is that the injected holes be 45 transported across the charge transport layer in a short time; shorter than the time duration between the exposure and development stations in an imaging device. The transit time across the transport layer is determined by the charge carrier mobility in the transport layer. The charge carrier mobility is 50 the velocity per unit field and has dimensions of  $\text{cm}^2/\text{volt sec}$ . The charge carrier mobility is a function of the structure of the charge transporting molecule, the concentration of the charge transporting molecule in the transport layer and the 55 electrically "inactive" binder polymer in which the charge transport molecule is dispersed.

Reproductive machines often utilize multilayered organic photoconductors and can also employ corotrons, scorotrons

or bias charging rolls to charge the photoconductors prior to imagewise exposure. Further, corotrons, scorotrons or bias transfer rolls may be utilized to transfer toner images from a photoreceptor to a receiving member. Bias transfer rolls for charging purposes have the advantage that they generally emit less ozone than corotrons and scorotrons. It has been found that as the speed and number of imaging of copiers, duplicators and printers are increased, bias transfer rolls and bias charge rolls can cause serious wear problems to the photoreceptors. Bias transfer rolls and bias charge rolls are known in the art. Bias transfer rolls, which are similar to bias charge rolls, are described, for example in U.S. Pat. No. 5,420,677, U.S. Pat. No. 5,321,476 and U.S. Pat. No. 5,303,014. The entire disclosures of these patents are incorporated herein by reference. As a consequence of the abrasive action of the bias transfer rolls and bias charge rollers, the operating lifetime of conventional photoreceptors is severely reduced. In a test conducted on a normally abrasion resistant non-crosslinked overcoated photoreceptor composition, introduction of bias transfer roll and bias charge roll subsystems causes a greater than eight fold increase in wear of the overcoated photoreceptor. The precise nature of the electrical/abrasive wearing away of the charge transport layer thickness is unknown, but it is theorized that some degradative process involving charge scission of the binder occurs, or in the case of arylamine hole transporting polymers, a reduction in chain lengths causes the polymers to lose their inherent strength.

As described above, one type of multilayered photoreceptor that has been employed as a belt in electrophotographic imaging systems comprises a substrate, a conductive layer, a charge blocking layer a charge generating layer, and a charge transport layer. The charge transport layer often comprises an activating small molecule dispersed or dissolved in a polymeric film forming binder. Generally, the polymeric film forming binder in the transport layer is electrically inactive by itself and becomes electrically active when it contains the activating molecule. The expression "electrically active" means that the material is capable of supporting the injection of photogenerated charge carriers from the material in the charge generating layer and is capable of allowing the transport of these charge carriers through the electrically active layer in order to discharge a surface charge on the active layer. The multilayered type of photoreceptor may also comprise additional layers such as an anticurl backing layer, an adhesive layer, and an overcoating layer. Although excellent toner images may be obtained with multilayered belt photoreceptors that are developed with dry developer powder (toner), it has been found that these same photoreceptors become unstable when employed with liquid development systems. These photoreceptors suffer from cracking, crazing, crystallization of active compounds, phase separation of activating compounds and extraction of activating compounds caused by contact with the organic carrier fluid, isoparaffinic hydrocarbons e.g. Isopar (Exxon Chemical Inc), commonly employed in liquid developer inks. These carrier fluids markedly degrade the mechanical integrity and electrical properties of the photoreceptor. More specifically, the organic carrier fluid of a liquid developer tends to leach out activating small molecules, such as the arylamine containing compounds typically used in the charge transport layers. Representative of this class of materials are: N,N'-diphenyl-N,N'-bis(3-methylphenyl)-[1,1'-biphenyl]4,4',diamine; bis-(4-diethylamino-2-methylphenyl)-phenylmethane; 2,5-bis-(4'-dimethylaminophenyl)-1,3,4,-oxadiazole; 1-phenyl-3-(4'-diethylaminostyryl)-5-(4"-diethylaminophenyl)-

pyrazoline; 1,1-bis-(4-(di-N,N'-p-methylphenyl)-aminophenyl)-cyclohexane; 4-diethylaminobenzaldehyde-1,1-diphenylhydrazone; 1,1-diphenyl-2(p-N,N-diphenyl amino phenyl)-ethylene; N-ethylcarbazole-3-carboxaldehyde-1-methyl-1phenylhydrazone. The leaching process results in crystallization of the activating small molecules, such as the aforementioned arylamine compounds, onto the photoreceptor surface and subsequent migration of arylamines into the liquid developer ink. In addition, the ink vehicle, typically a C<sub>10</sub>-C<sub>14</sub> branched hydrocarbon, induces the formation of cracks and crazes in the photoreceptor surface. These effects lead to copy defects and shortened photoreceptor life. The degradation of the photoreceptor manifests itself as increased background and other printing defects prior to complete physical photoreceptor failure. The leaching out of the activating small molecule also increases the susceptibility of the transport layer to solvent/stress cracking when the belt is parked over a belt support roller during periods of non-use. Some carrier fluids may also promote phase separation of the activating small molecules, such as arylamine compounds, in the transport layers, particularly when high concentrations of the arylamine compounds are present in the transport layer binder. Phase separation of activating small molecules also adversely alters the electrical and mechanical properties of a photoreceptor. Similarly, single layer photoreceptors having a single active layer comprising photoconductive particles dispersed in a charge transport film forming binder are also vulnerable to the same degradation problems encountered by the previously described multilayered type of photoreceptor when exposed to liquid developers. Although flexing is normally not encountered with rigid, cylindrical, multilayered photoreceptors which utilize charge transport layers containing activating small molecules dispersed or dissolved in a polymeric film forming binder, electrical degradation are similarly encountered during development with liquid developers. Sufficient degradation of these photoreceptors by liquid developers can occur in less than two hours as indicated by leaching of the small molecule and cracking of the matrix polymer film. Continued exposure for several days severely damages the photoreceptor. Thus, in advanced imaging systems utilizing multilayered belt photoreceptors exposed to liquid development systems, cracking and crazing have been encountered in critical charge transport layers during belt cycling. Cracks developing in charge transport layers during cycling can be manifested as print-out defects adversely affecting copy quality. Furthermore, cracks in the photoreceptor pick up toner particles which cannot be removed in the cleaning step and may be transferred to the background in subsequent prints. In addition, crack areas are subject to delamination when contacted with blade cleaning devices thus limiting the options in electrophotographic product design.

Photoreceptors have been developed which comprise charge transfer complexes prepared with polymeric molecules. For example, charge transfer complexes formed with polyvinyl carbazole are disclosed in U.S. Pat. No. 4,047,948, U.S. Pat. No. 4,346,158 and U.S. Pat. No. 4,388,392. Photoreceptors utilizing polyvinyl carbazole layers, as compared with current photoreceptor requirements, exhibit relatively poor xerographic performance in both electrical and mechanical properties. Polymeric arylamine molecules prepared from the condensation or di-secondary amine with a di-iodo aryl compound are disclosed in European Patent Publication 34,425, published Aug. 26, 1981, issued May 16, 1984. Since these polymers are extremely brittle and form films which are very susceptible to physical damage,

their use in a flexible belt configuration is precluded. Thus, in advanced imaging systems utilizing multilayered belt photoreceptors exposed to liquid development, cracking and crazing have been encountered in critical charge transport layers during belt cycling. Still other arylamine charge transporting polymers such as those disclosed in U.S. Pat. No. 4,806,444, U.S. Pat. No. 4,806,443, U.S. Pat. No. 4,935,487, and U.S. Pat. No. 5,030,532 are vulnerable to reduced life because of the highly abrasive conditions presented by imaging systems utilizing bias transfer rolls and/or bias charge rollers.

Protective overcoatings can be somewhat helpful against abrasion. However, most protective overcoatings also fail early when subjected to the highly abrasive conditions presented by imaging systems utilizing bias transfer rolls and/or bias charge rollers. Moreover, many overcoatings tend to accumulate residual charge during cycling. This can cause a condition known as cycle-up in which the residual potential continues to increase with multi-cycle operation. This can give rise to increased densities in the background areas of the final images.

Drum machines employing small diameter drum blanks coated with organic photoreceptors are even more susceptible to degradation since it takes many revolutions of the drum to make a single print. The wear in machines employing bias charging rolls (BCR) and bias transfer rolls (BTR) might be as much as 10 micrometers in less than 100,000 revolutions which could translate to as few as 10,000 prints. There is an urgent need for an effective, wear resistant overcoat for these drums. Since the drums are invariably dip coated, one of the requirements for the overcoat material requirements is ease and economical synthesis of the materials and a coating solution pot life of several weeks. Pot life is the life of the coating slurry without changes in its properties so that the same mixture can be used for several weeks. With coating compositions that ultimately crosslink and provide wear protection, there is a danger of initiation of crosslinking in the pot itself rendering the remaining material in the pot useless for coating. Since the unused material must be discarded and the pot cleaned or replaced, this waste of material and effort has a significant negative impact on the manufacturing cost. In some instances phase separation of different constituents in the overcoat slurry and or changes in the viscosity impact the pot life of the coating slurry.

#### INFORMATION DISCLOSURE STATEMENT

U.S. Pat. No. 4,871,634 to W. Limburg et.al., issued Oct. 3, 1989—A hydroxylarylamine compound, represented by a specific formula, is disclosed as employable in photoreceptors. The hydroxylarylamine compound can be used as an overcoating with the hydroxylarylamine compound bonded to a resin capable of hydrogen bonding such as a polyamide possessing alcohol solubility.

U.S. Pat. No. 5,368,967 to R. Schank et. al., Nov. 29, 1994—An electrophotographic imaging member is disclosed comprising a substrate, a charge generating layer, a charge transport layer, and an overcoat layer comprising a small molecule hole transporting arylamine having at least two hydroxy functional groups, a hydroxy or multihydroxy triphenyl methane and a polyamide film forming binder capable of forming hydrogen bonds with the hydroxy functional groups of the hydroxy arylamine and the hydroxy or multihydroxy triphenyl methane. This overcoat layer may be fabricated using an alcohol solvent. This electrophotographic imaging member may be utilized in an electrophotographic imaging process.

U.S. Pat. No. 5,681,679, to R. Schank et. al.—A flexible electrophotographic imaging member is disclosed including a supporting substrate and a resilient combination of at least one photoconductive layer and an overcoating layer, the at least one photoconductive layer comprising a hole transporting arylamine siloxane polymer and the overcoating comprising a crosslinked polyamide doped with a dihydroxy amine. This imaging member may be utilized in an imaging process including forming an electrostatic latent image on the imaging member, depositing toner particles on the imaging member in conformance with the latent image to form a toner image, and transferring the toner image to a receiving member.

U.S. Pat. No. 5,709,974 to H. Yuh et. al.—An electrophotographic imaging member is disclosed including a charge generating layer, a charge transport layer and an overcoating layer, the transport layer including a charge transporting aromatic diamine molecule in a polystyrene matrix and the overcoating layer including a hole transporting hydroxy arylamine compound having at least two hydroxy functional groups and a polyamide film forming binder capable of forming hydrogen bonds with the hydroxy functional groups of the hydroxy arylamine compound. This imaging member is utilized in an imaging process.

U.S. Pat. No. 5,702,854 to Shank et al.—An electrophotographic imaging member is disclosed including a supporting substrate coated with at least a charge generating layer, a charge transport layer and an overcoating layer, said overcoating layer comprising a dihydroxy arylamine dissolved or molecularly dispersed in a crosslinked polyamide matrix. The overcoating layer is formed by crosslinking a crosslinkable coating composition including a polyamide containing methoxy methyl groups attached to amide nitrogen atoms, a crosslinking catalyst and a dihydroxy amine, and heating the coating to crosslink the polyamide. The electrophotographic imaging member may be imaged in a process involving uniformly charging the imaging member, exposing the imaging member with activating radiation in image configuration to form an electrostatic latent image, developing the latent image with toner particles to form a toner image, and transferring the toner image to a receiving member.

U.S. Pat. No. 5,670,291 to Ward et al., Sep. 23, 1997—A process for fabricating an electrophotographic imaging member is disclosed including

providing a substrate coated with at least one photoconductive layer,  
applying a coating composition to the photoconductive layer by dip coating to form a wet layer, the coating composition comprising finely divided amorphous silica particles, a dihydroxy amine charge transport material, an aryl charge transport material that is different from the dihydroxy amine charge transport material, a crosslinkable polyamide containing methoxy groups attached to amide nitrogen atoms and a crosslinking catalyst, at least one solvent for the hydroxy amine charge transport material, aryl charge transport material that is different from the dihydroxy amine charge transport material and the crosslinkable polyamide, and

heating the wet layer to crosslink the polyamide and remove the solvent to form a dry layer in which the dihydroxy amine charge transport material and the aryl charge transport material are molecularly dispersed in a crosslinked polyamide matrix.

U.S. Pat. No. 5,612,157 issued to Yuh et al. on Mar. 18, 1997—An electrophotographic imaging member is dis-

closed including a substrate, a hole blocking layer comprising hydrolyzed metal alkoxide or aryloxide molecules and a film forming alcohol soluble nylon polymer, an optional interface adhesive layer, a charge generating layer, and a charge transport layer.

CROSS REFERENCE TO RELATED APPLICATIONS

This application is related to the following U.S. patent applications:

U.S. patent application Ser. No. 09/182,602, filed concurrently herewith in the names of Yanus et al., entitled "OVERCOATING COMPOSITIONS, OVERCOATED PHOTORECEPTORS, AND METHODS OF FABRICATING AND USING OVERCOATED PHOTORECEPTORS"—An electrophotographic imaging member including a supporting substrate coated with at least photoconductive layer, a charge transport layer and an overcoating layer, the overcoating layer including a hydroxy functionalized aromatic diamine and a hydroxy functionalized triarylamine dissolved or molecularly dispersed in a crosslinked polyamide matrix, the crosslinked polyamide prior to crosslinking being selected from the group consisting of materials represented by the following Formulae I and II:

I



wherein:

n is a positive integer sufficient to achieve a weight average molecular weight between about 5000 and about 100,000,

R is an alkylene unit containing from 1 to 10 carbon atoms,

between 1 and 99 percent of the R<sub>2</sub> sites are —H, and the remainder of the R<sub>2</sub> sites are —CH<sub>2</sub>—O—CH<sub>3</sub>, and

II



wherein:

m is a positive integer sufficient to achieve a weight average molecular weight between about 5000 and about 100,000,

R<sub>1</sub> and R are independently selected from the group consisting of alkylene units containing from 1 to 10 carbon atoms, and

between 1 and 99 percent of the R<sub>3</sub> and R<sub>4</sub> sites are —H, and

the remainder of the R<sub>3</sub> and R<sub>4</sub> sites are —CH<sub>2</sub>—O—CH<sub>3</sub>.

Coating compositions for the overcoating layer of this invention as well as methods of making and using the overcoated photoreceptor are also disclosed.

Thus, there is a continuing need for photoreceptors having improved resistance to abrasive cycling conditions and

without an attendant increased densities in the background areas of the final images, and without attendant cyclic instabilities. There is also continuing need for improved photoconductors for use in a liquid ink environment. There is also a continuing need for overcoat materials that are easily and economically synthesizable and scalable. Further, there is a continuing need for overcoat materials that have a long pot life when made into a solution for dip coating. Additionally, there is a continuing need for overcoat materials that employ catalysts free of acid to crosslink the overcoat.

SUMMARY OF THE INVENTION

It is, therefore, an object of the present invention to provide an improved electrophotographic imaging member which overcomes the above-noted deficiencies.

It is yet another object of the present invention to provide an improved electrophotographic imaging member capable of longer cycling life under abrasive imaging conditions.

It is yet another object of the present invention to provide an improved electrophotographic imaging member capable of longer cycling life under abrasive toner/cleaning blade interactions.

It is still another object of the present invention to provide an improved electrophotographic imaging member that is stable against increasing residual voltages with repetitive use, i.e., cycle-up.

It is another object of the present invention to provide an improved electrophotographic imaging member that resists cracking in a liquid development environment.

It is yet another object of the present invention to provide an improved electrophotographic imaging member exhibiting resistance against rough handling in a copier image cycling environment.

It is yet another object of the present invention to provide an improved electrophotographic imaging member exhibiting resistance against rough handling during installation and service.

It is yet another object of the present invention to provide an improved electrophotographic imaging member with an overcoat fabricated from easily and economically synthesizable materials.

It is yet another object of the present invention to provide an improved electrophotographic imaging member with an overcoat applied with a dip coating solution having a long pot life.

It is yet another object of the present invention to provide an improved electrophotographic imaging member with an overcoat applied as dip coating solution which uses a catalyst free of acid for crosslinking.

The foregoing objects and others are accomplished in accordance with this invention by

providing an electrophotographic imaging member comprising  
a supporting substrate coated with  
at least one photoconductive layer, and  
an overcoating layer, the overcoating layer comprising  
a hydroxy functionalized aromatic diamine and  
a hydroxy functionalized triarylamine dissolved or  
molecularly dispersed in  
a crosslinked acrylated polyamide matrix, the hydroxy functionalized triarylamine being a compound different from the polyhydroxy functionalized aromatic diamine, the crosslinked polyamide prior to

crosslinking being selected from the group consisting of materials represented by the following Formulae I and II:



wherein:

n is a positive integer sufficient to achieve a weight average molecular weight between about 5000 and about 100,000,

R is an alkylene group containing from 1 to 10 carbon atoms, between 1 and 99 percent of the R<sub>2</sub> sites are



wherein

X is selected from the group consisting of —H (acrylate), —CH<sub>3</sub> (methacrylate), alkyl and aryl, and

the remainder of the R<sub>2</sub> sites are selected from the group consisting of —H, —CH<sub>2</sub>OCH<sub>3</sub>, and —CH<sub>2</sub>OH, and



wherein:

m is a positive integer sufficient to achieve a weight average molecular weight between about 5000 and about 100000,

R and R<sub>1</sub> are independently selected from the group consisting of alkylene units containing from 1 to 10 carbon atoms;

between 1 and 99 percent of R<sub>3</sub> and R<sub>4</sub> are independently selected from the group consisting of



wherein

X is selected from the group consisting of hydrogen, alkyl, aryl and alkylaryl, wherein the alkyl groups contain 1 to 10 carbon atoms and the aryl groups contain 1 to 3 alkyl groups,

y is an integer between 1 and 10, and

the remainder of the R<sub>3</sub> and R<sub>4</sub> groups are selected from the group consisting of —H, —CH<sub>2</sub>OH, —CH<sub>2</sub>OCH<sub>3</sub>, and —CH<sub>2</sub>OC(O)—C(X)=CH<sub>2</sub>.

The overcoating layer is formed by crosslinking a crosslinkable coating composition comprising an alcohol soluble

acrylated polyamide containing acryloxy-methyl or acryloxyalkyl-methyl groups attached to amide nitrogen atoms, a crosslinking catalyst and a mixture of a hydroxy functionalized aromatic diamine with a hydroxy functionalized triarylamine. The electrophotographic imaging member may be imaged in a process involving uniformly charging the imaging member, exposing the imaging member with activating radiation in image configuration to form an electrostatic latent image, developing the latent image with toner particles to form a toner image, and transferring the toner image to a receiving member.

Electrophotographic imaging members are well known in the art. Electrophotographic imaging members may be prepared by any suitable technique. Typically, a flexible or rigid substrate is provided with an electrically conductive surface. At least one photoconductive layer is applied to the electrically conductive surface. Thus, as well known in the art of electrophotography, a single photoconductive layer comprising photoconductive particles dispersed in an electrically active matrix may be applied or a plurality of photoconductive layers, such as a charge generating layer and a separate charge transport layer may be applied to the electrically conductive surface. A charge blocking layer may optionally be applied to the electrically conductive surface prior to the application of the at least one photoconductive layer desired, an adhesive layer may be utilized between the charge blocking layer and the at least one photoconductive layer. Usually the charge generation layer is applied onto the blocking layer and a charge transport layer is formed on the charge generation layer. This structure may have the charge generation layer on top of or below the charge transport layer.

The substrate may be opaque or substantially transparent and may comprise any suitable material having the required mechanical properties. Accordingly, the substrate may comprise a layer of an electrically non-conductive or conductive material such as an inorganic or an organic composition. As electrically non-conducting materials here may be employed various resins known for this purpose including polyesters, polycarbonates, polyamides, polyurethanes, and the like which are flexible as thin webs. An electrically conducting substrate may be any metal, for example, aluminum, nickel, steel, copper, and the like or a polymeric material, as described above, filled with an electrically conducting substance, such as carbon, metallic powder, and the like or an organic electrically conducting material. The electrically insulating or conductive substrate may be in the form of an endless flexible belt, a web, a rigid cylinder, a sheet and the like.

The thickness of the substrate layer depends on numerous factors, including strength desired and economical considerations. Thus, for a drum, this layer may be of substantial thickness of, for example, up to many centimeters or of a minimum thickness of less than a millimeter. Similarly, a flexible belt may be of substantial thickness, for example, about 250 micrometers, or a minimum thickness less than 50 micrometers, provided there are no adverse effects on the final electrophotographic device.

In embodiments where the substrate layer is not conductive, the surface thereof may be rendered electrically conductive by an electrically conductive coating. The conductive coating may vary in thickness over substantially wide ranges depending upon the optical transparency, degree of flexibility desired, and economic factors. Accordingly, for a flexible photoresponsive imaging device, the thickness of the conductive coating may be between about 20 angstroms to about 200 angstroms for an optimum

combination of electrical conductivity, flexibility and light transmission. The flexible conductive coating may be an electrically conductive metal layer formed, for example, on the substrate by any suitable coating technique, such as a vacuum depositing technique or electrodeposition. Typical metals include aluminum, zirconium, niobium, tantalum, vanadium and hafnium, titanium, nickel, stainless steel, chromium, tungsten, molybdenum, and the like.

An optional hole blocking layer may be applied to the substrate. Any suitable and conventional blocking layer capable of forming an electronic barrier to holes between the adjacent photoconductive layer and the underlying conductive surface of the substrate may be utilized.

An optional adhesive layer may be applied to the hole blocking layer. Any suitable adhesive layer well known in the art may be utilized. Typical adhesive layer materials include, for example, polyesters, polyurethanes, and the like. Satisfactory results may be achieved with adhesive layer thickness between the 0.05 micrometer (500 angstroms) and about 0.3 micrometer (3,000 angstroms). Conventional techniques for applying an adhesive layer coating mixture to the charge blocking layer include spraying, dip coating, roll coating, wire wound rod coating, gravure coating, bird applicator coating, and the like. Drying of the deposited coating may be affected by any suitable conventional technique such as oven drying, infrared radiation drying, air drying and the like.

Any suitable polymeric film forming binder material may be employed as the matrix in the charge generating (photogenerating) binder layer. Typical polymeric film forming materials include those described, for example, in U.S. Pat. No. 3,121,006, the entire disclosure of which is incorporated herein by reference. Thus, typical organic polymeric film forming binders include thermoplastic and thermosetting resins such as polycarbonates, polyesters, polyamides, polyurethanes, polystyrenes, polyarylethers, polyarylsulfones, polybutadienes, polysulfones, polyethersulfones, polyethylenes, polypropylenes, polyimides, polymethylpentenes, polyphenylene sulfides, polyvinyl acetate, polysiloxanes, polyacrylates, polyvinyl acetals, polyamides polyimides, amino resins, phenylene oxide resins, terephthalic acid resins, phenoxy resins, epoxy resins, phenolic resins, polystyrene and acrylonitrile copolymers, polyvinylchloride, vinylchloride and vinyl acetate copolymers, acrylate copolymers, alkyd resins, cellulosic film formers, poly(amideimide), styrene-butadiene copolymers, vinylidenechloride-vinylchloride copolymers, vinylacetate-vinylidenechloride copolymers, styrene-alkyd resins, polyvinylcarbazole, and the like. These polymers may be block, random or alternating copolymers.

The photogenerating composition or pigment is present in the resinous binder composition in various amounts. Generally, however, from about 5 percent by volume to about 90 percent by volume of the photogenerating pigment is dispersed in about 10 percent by volume to about 95 percent by volume of the resinous binder, and preferably from about 20 percent by volume to about 30 percent by volume of the photogenerating pigment is dispersed in about 70 percent by volume to about 80 percent by volume of the resinous binder composition. In one embodiment about 8 percent by volume of the photogenerating pigment is dispersed in about 92 percent by volume of the resinous binder composition. The photogenerator layers can also be fabricated by vacuum sublimation in which case there is no binder.

Any suitable and conventional technique may be utilized to mix and therefore apply the photogenerating layer coating

mixture. Typical application techniques include spraying, dip coating, roll coating, wire wound rod coating, vacuum sublimation and the like. For some applications, the generator layer may be fabricated in a dot or line pattern. Removing 5 of the solvent from a solvent coated layer may be effected by any suitable conventional technique such as oven drying, infrared radiation drying, air drying and the like.

The charge transport layer may comprise a charge transporting small molecule dissolved or molecularly dispersed 10 in a film forming electrically inert polymer such as a polycarbonate. The term "dissolved" as employed herein is defined herein as forming a solution in which the small molecule is dissolved in the polymer to form a homogeneous phase. The expression "molecularly dispersed" as used 15 herein is defined as a charge transporting small molecule dispersed in the polymer, the small molecules being dispersed in the polymer on a molecular scale. Any suitable charge transporting or electrically active small molecule may be employed in the charge transport layer of this 20 invention. The expression charge transporting "small molecule" is defined herein as a monomer that allows the free charge photogenerated into the transport layer to be transported across the transport layer. Typical charge transporting small molecules include, for example, pyrazolines such as 25 1-phenyl-3-(4'-diethylamino styryl)-5-(4"-diethylamino phenyl) pyrazoline, diamines such as N,N'-diphenyl-N,N'-bis(3-methylphenyl)-(1,1-biphenyl)-4,4'-diamine, hydrazones such as N-phenyl-N-methyl-3-(9-ethyl) carbazyl hydrazone and N,N-diethyl amino benzaldehyde-1,2-diphenyl hydrazone, and oxadiazoles such as 2,5-bis (4-N, 30 N'-diethylaminophenyl)-1,2,4-oxadiazole, stilbenes and the like. However, to avoid cycle-up, the charge transport layer should be substantially free of triphenyl methane. As indicated above, suitable electrically active small molecule 35 charge transporting compounds are dissolved or molecularly dispersed in electrically inactive polymeric film forming materials. A small molecule charge transporting compound that permits injection of holes from the pigment into the charge generating layer with high efficiency and transports 40 them across the charge transport layer with very short transit times is N,N'-diphenyl-N,N'-bis(3-methylphenyl)-(1,1'-biphenyl)-4,4'-di-amine.

Any suitable electrically inert polymeric binder may be used to disperse the electrically active molecule in the 45 charge transport layer such as poly (4,4'-isopropylidene-diphenylene) carbonate (also referred to as bisphenol-A-polycarbonate), poly (4,4'-isopropylidene-diphenylene) carbonate, poly (4,4'-diphenyl-1/1'-cyclohexane carbonate), and the like. Other typical inactive resin binders include 50 polyester, polyarylate, polyacrylate, polyether, polysulfone, and the like. Molecular weights can vary, for example, from about 20,000 to about 150,000. However, weight average molecular weights outside this range may be utilized where suitable.

Instead of a small molecule charge transporting compound dissolved or molecularly dispersed in an electrically inert polymeric binder, the charge transport layer may comprise any suitable charge transporting polymer. A typical charge transporting polymers is one obtained from the 55 condensation of N,N'-diphenyl-N,N'-bis (3-hydroxy phenyl)-[1-1'-biphenyl]-4,4'-diamine and diethylene glycol bischloroformate such as disclosed in the U.S. Pat. No. 4,870,644 and U.S. Pat. No. 5,028,687, the entire disclosures of these patents being incorporated herein by reference. Another typical charge transporting polymer is poly (N,N'-bis-(3-oxyphenyl)-N,N'-diphenyl [1,1'-biphenyl]-4, 60 4'-diaminobacoyl) polyethercarbonate obtained from the 65

## 13

condensation of N,N'-diphenyl-N,N'-bis (3-hydroxy phenyl)-[1,1'-biphenyl]-4,4'-diamine and sebacoyl chloride.

Any suitable and conventional technique may be utilized to mix and thereafter apply the charge transport layer coating mixture to the charge generating layer. Typical application techniques include spraying, dip coating, roll coating, wire wound rod coating, and the like. Drying of the deposited coating may be affected by any suitable conventional technique such as oven drying, infrared radiation drying, air drying and the like.

Generally, the thickness of the charge transport layer is between about 10 and about 50 micrometers, but thicknesses outside this range can also be used. The hole transport layer should be an insulator to the extent that the electrostatic charge placed on the hole transport layer is not conducted in the absence of illumination at a rate sufficient to prevent formation and retention of an electrostatic latent image thereon. In general, the ratio of the thickness of the hole transport layer to the charge generator layers is preferably maintained from about 2:1 to 200:1 and in some instances as great as 400:1. In other words, the charge transport layer is substantially non-absorbing to visible light or radiation in the region of intended use but is electrically "active" in that it allows the injection of photogenerated holes from the photoconductive layer, i.e., charge generation layer, and allows these holes to be transported through itself to selectively discharge a surface charge on the surface of the active layer.

The overcoat layer of this invention comprises a mixture of a hydroxy functionalized aromatic diamine with a hydroxy functionalized triarylamine dissolved or molecularly dispersed in a crosslinked acrylated polyamide matrix. The overcoat layer is formed from a crosslinkable coating composition comprising an alcohol soluble acrylated polyamide containing acyloxy-methyl or acyloxyalkyl-methyl groups attached to amide nitrogen atoms, an optional crosslinking catalyst, and a mixture of a hydroxy functionalized aromatic diamine with a hydroxy functionalized triarylamine.

Any suitable hole insulating film forming alcohol soluble acrylated polyamide polymer having acyloxy-methyl groups or acyloxyalkyl-methyl groups attached to the nitrogen atoms of amide groups in the polymer backbone prior to crosslinking may be employed in the overcoating of this invention. A preferred alcohol soluble polyamide polymer having acyloxy-methyl groups or acyloxyalkyl-methyl groups attached to the nitrogen atoms of amide groups in the polymer backbone prior to crosslinking is selected from the group consisting of materials represented by the following Formulae I and II:



I

wherein:

n is a positive integer sufficient to achieve a weight average molecular weight between about 5000 and about 100,000,

## 14

R is an alkylene group containing 1 to 10 carbon atoms,

and

between 1 and 99 percent of the R2 sites are



wherein

X is selected from the group consisting of H (acrylate),

CH3 (methacrylate), alkyl and aryl, and

the remainder of the R2 sites are selected from the group consisting of H, -CH2OCH3, and -CH2OH, and

II



wherein:

m is a positive integer sufficient to achieve a weight average molecular weight of between about 5000 and about 100000,

R and R1 are independently selected from the group consisting of alkylene groups containing 1 to 10 carbon atoms,

between 1 and 99 percent of R3 and R4 are independently selected from the group consisting of



wherein

X is selected from the group consisting of hydrogen, alkyl, aryl and alkylaryl, wherein the alkyl groups contain 1 to 10 carbon atoms and the aryl groups contain 1 to 3 alkyl groups,

y is an integer between 1 and 10 and

the remainder of the R3 and R4 groups are selected from the group consisting of -H, -CH2OH, -CH2OCH3, and -CH2OC(O)-C(X)=CH2.

Between about 1 mole percent and about 50 mole percent of the total number of repeat units of the polyamide should contain acyloxy-methyl or acyloxyalkyl-methyl groups attached to the nitrogen atoms of amide groups. These acrylated polyamides should form solid films when dried prior to crosslinking. The acrylated polyamide should also be soluble, prior to crosslinking, in the alcohol solvents employed. Regarding Formula II, optimum results are achieved when n is less than 6 and R and R1 comprise between about 20 and 60 percent of the total number of alkylene groups.

A preferred acrylated polyamide is an acyloxyethyl modified Elvamide, (unmodified Elvamide being available from DuPont de Nemours & Co) represented by the following formula:

Structure 1



wherein

R<sub>1</sub>, R<sub>2</sub> and R<sub>3</sub> are alkylene groups containing 1 to 10 carbon atoms, and

n is a positive integer sufficient to achieve a weight average molecular weight between about 5000 and about 100000.

Optimum results are achieved when R<sub>1</sub>, R<sub>2</sub> and R<sub>3</sub> in Structure 1 are alkylene groups containing less than 6 carbon atoms and comprise between 20 and 60 percent of the total number of alkyl groups.

Another preferred acrylated polyamide is acryloxyethoxy-methyl modified Elvamide, (unmodified Elvamide being available from DuPont de Nemours & Co) represented by the following formula:

5



10

wherein R<sub>1</sub>, R<sub>2</sub> and R<sub>3</sub> are alkyl groups containing 1 to 10 carbon atoms,

Optimum results are achieved when the R<sub>1</sub>, R<sub>2</sub> and R<sub>3</sub> in Structure 2 are alkylene groups containing less than 6 carbon atoms and comprise between about 20 and 60 percent of the total number of alkyl groups.

Elvamide was chemically modified by reaction with paraformaldehyde and acrylic acid to form acryloxy-methyl modified Elvamide which is represented by Structure 1.

Alternatively, acryloxyethoxy-methyl modified Elvamide which is represented by Structure 2, was formed when the same reaction is repeated in the presence of 2-hydroxyethylacrylate.

20 Acrylated polyamides differ from Luckamide disclosed in the prior art, the Luckamide being an alcohol soluble methoxy-methylated polyamide available from Dai Nippon Ink with the following structure:

25

Structure 2



wherein

45

R<sub>1</sub>, R<sub>2</sub> and R<sub>3</sub> are alkylene groups containing 1 to 10 carbon atoms,

n is a positive integer sufficient to achieve a weight average molecular weight between about 5000 and about 100000.

Optimum results are achieved when the R<sub>1</sub>, R<sub>2</sub> and R<sub>3</sub> in Structure 2 are alkylene groups containing less than 6 carbon atoms and comprise about 40 percent of the total number of alkyl groups. Typical alcohols in which the acrylated polyamide is soluble include, for example, butanol, ethanol, methanol, and the like.

50



55

Typical alcohol soluble, film-forming polyamide polymers having methoxy methyl groups attached to the nitrogen atoms of amide groups in the polymer backbone prior to crosslinking include, for example, hole insulating polymer, for example, Luckamide 5003 from Dai Nippon Ink, Nylon 8 with methylmethoxy pendant groups, CM4000 from Toray Industries, Ltd. and CM8000 from Toray Industries, Ltd., other N-methoxymethylated polyamides, such as those prepared according to the method described in Sorenson and Campbell "Preparative Methods of Polymer Chemistry" second edition, pg. 76, John Wiley & Sons Inc. 1968, and the like and mixtures thereof. These polyamides can be alcohol soluble, for example, with polar functional groups, such as methoxy, ethoxy and hydroxy groups, pendant from the

60

65 It should be noted that polyamides, such as the Elvamides from DuPont de Nemours & Co., do not contain methoxy methyl groups attached to the nitrogen atoms of amide groups in the polymer backbone.

65

polymer backbone. It should be noted that polyamides, such as Elvamides from DuPont de Nemours & Co., do not contain methoxy methyl groups attached to the nitrogen atoms of amide groups in the polymer backbone.

The overcoating layer of this invention preferably comprises between about 50 percent by weight and about 98 percent by weight of the crosslinked film forming crosslinkable alcohol soluble polyamide polymer having acryloxy-methyl or acryloxyalkyl-methyl groups attached to the nitrogen atoms of the amide groups in the polymer backbone, based on the total weight of the overcoating layer after crosslinking and drying. These film forming acrylated polyamides are also soluble in a solvent to facilitate application by conventional coating techniques. Typical solvents include, for example, butanol, propanol, methanol, butyl acetate, ethanol, cyclohexanone, tetrahydrofuran, methyl ethyl ketone, and the like and mixtures thereof. Crosslinking is achieved by a variety of mechanisms: (1) a thermal, acid catalyzed condensation reaction, and/or (2) the photo and/or thermal polymerization of acrylate groups on the polymers. Crosslinking is accomplished by heat alone or by heating in the presence of a catalyst. The thermal curing of the acrylated Elvamides can be accelerated with free radical initiators such as azobisisobutyronitrile (AIBN). By contrast, the use of benzoyl peroxide results in oxidation of hole transporting arylamine molecules which are conductive and therefore undesirable. Any suitable catalyst may be employed. Typical acid catalysts include, for example, oxalic acid, maleic, carboxylic, ascorbic, malonic, succinic, tartaric, citric, p-toluenesulfonic acid, methanesulfonic acid, and the like and mixtures thereof. Catalysts that transform into a gaseous product during the crosslinking reaction are preferred because they escape the coating mixture and leave no residue that might adversely affect the electrical properties of the final overcoating. A typical gas forming catalyst is, for example, oxalic acid. The photochemical cure can be accomplished with any suitable well known photochemical initiators such as Michler's ketone, and the like. The temperature used for crosslinking varies with the specific catalyst and heating time utilized and the degree of crosslinking desired. Generally, the degree of crosslinking selected depends upon the desired flexibility of the final photoreceptor. For example, complete crosslinking may be used for rigid drum or plate photoreceptors. However, partial crosslinking is preferred for flexible photoreceptors having, for example, web or belt configurations. The degree of crosslinking can be controlled by the relative amount of catalyst employed. The amount of catalyst to achieve a desired degree of crosslinking will vary depending upon the specific acrylated polyamide, catalyst, temperature and time used for the reaction. A typical crosslinking temperature used for acrylated polyamide with oxalic acid as a catalyst is about 120° C. for 30 minutes. A typical concentration of oxalic acid is between about 5 and about 10 weight percent based on the weight of acryloxy polyamide. Alternatively, between about 0.5 and about 10 weight percent azobisisobutyronitrile can be used to crosslink the acrylated polyamide by the free-radical polymerization of acrylate groups at about 120° C. within about 30 minutes. After crosslinking, the overcoating is substantially insoluble in the solvent in which it was soluble prior to crosslinking. Thus, no overcoating material will be removed when rubbed with a cloth soaked in the solvent. Crosslinking results in the development of a three dimensional network which immobilizes the hydroxy functionalized transport molecule in the overcoat.

The overcoating of this invention includes a mixture of a hydroxy functionalized aromatic diamine with a hydroxy

functionalized triarylamine. Preferably, the hydroxy functionalized aromatic diamine is represented by the following formula:



wherein

10 Z is selected from the group consisting of:



20 n is 0 or 1,

Ar is selected from the group consisting of:



25 R is selected from the group consisting of —CH<sub>3</sub>, —C<sub>2</sub>H<sub>5</sub>, —C<sub>3</sub>H<sub>7</sub>, and —C<sub>4</sub>H<sub>9</sub>,

Ar' is selected from the group consisting of:



30 X is selected from the group consisting of:



35 s is 0, 1 or 2

40 the hydroxy functionalized aromatic diamine compound being free of any direct conjugation between —OH groups and the nearest nitrogen atom through one or more aromatic rings.

45 Typical hydroxy functionalized aromatic diamines include, for example:

N,N'-diphenyl-N,N'-bis(3-hydroxyphenyl)-[1,1'-biphenyl]-4,4'-diamine;

N,N,N',N'-tetra(3-hydroxyphenyl)-[1,1'-biphenyl]-4,4'-diamine;

N,N'-diphenyl-N,N'-bis(3-hydroxyphenyl)-[1,1':4',1"-terphenyl]-4,4"-diamine,

## 19

N,N'-diphenyl-N,N'-bis(4-hydroxyphenyl)-[1,1'-biphenyl]-4,4"-diamine,  
N,N,N',N'-tetra(4-hydroxyphenyl)-[1,1'-biphenyl]-4,4'-diamine;

A specific preferred hydroxy functionalized aromatic diamine compound is N,N'-diphenyl-N,N'-bis(3-hydroxyphenyl)-[1,1'-biphenyl]-4,4'-diamine and is represented by the formula:



Examples of these polyhydroxy functionalized aromatic diamines are described, for example, in U.S. Pat. No. 4,871,634, the entire disclosure thereof being incorporated herein by reference.

The hydroxy functionalized triarylamine component of the mixture of hydroxy functionalized molecules invention is a compound different from the polyhydroxy functionalized aromatic diamine. Thus, for example, the hydroxy functionalized triarylamine compound contains a single nitrogen atom whereas the polyhydroxy functionalized aromatic diamine contains two nitrogen atoms. The hydroxy functionalized triarylamine compound may be represented by the formula:



wherein

Ar is selected from the group consisting of:



R is selected from the group consisting of  $-\text{CH}_3$ ,  $-\text{C}_2\text{H}_5$ ,  $-\text{C}_3\text{H}_7$  and  $-\text{C}_4\text{H}_9$ ,

Ar' and Ar" being independently selected from the group consisting of:



R is selected from the group consisting of  $-\text{CH}_3$ ,  $-\text{C}_2\text{H}_5$ ,  $-\text{C}_3\text{H}_7$  and  $-\text{C}_4\text{H}_9$ ,

the hydroxy functionalized triarylamine compound being free of any direct conjugation between the  $-\text{OH}$  groups and the nearest nitrogen atom through one or more aromatic rings.

## 20

Typical hydroxy functionalized triarylamine compounds of this invention include, for example: N-(3-hydroxyphenyl)-N-(4-methylphenyl)-N-phenyl amine;

- 5 N-(3-hydroxyphenyl)-N-bis(4-methylphenyl)amine
- N,N-di(3-hydroxyphenyl)-m-toluidine;
- 1,1-bis-[4-(di-N,N-m-hydroxypyphenyl)-aminophenyl]-cyclohexane;
- 1,1-bis[4-(N-m-hydroxyphenyl)-4-(N-phenyl)-aminophenyl]-cyclohexane;
- 10 N,N-di(4-hydroxyphenyl)-m-toluidine;
- 1,1-bis-[4-di-N,N-p-hydroxypyphenyl)-aminophenyl]-cyclohexane;
- Bis-N,N-[4'-hydroxy-4-(1,1'-biphenyl)]-aniline
- Bis-N,N-[2'-hydroxy-4-(1,1'-biphenyl)]-aniline

15 Two specific hydroxy functionalized triarylamine compounds are N-(3-hydroxyphenyl)-N-(4-methylphenyl)-N-phenyl amine (PTAP) and N-(3-hydroxyphenyl)-N-bis(4-methylphenyl)amine (DTAP) and are represented by the formulae:



and mixtures thereof.

The total concentration of hydroxy functionalized aromatic diamine and hydroxy functionalized triarylamine in the overcoat can be between about 3 percent and about 75 percent by weight based on the total weight of the dried overcoat. Preferably, the total concentration of hydroxy functionalized aromatic diamine and hydroxy functionalized triarylamine in the overcoat layer is between about 30 percent by weight and about 60 percent by weight based on the total weight of the dried overcoat. When less than about 30 percent by weight of hydroxy functionalized aromatic diamine and hydroxy functionalized triarylamine is present in the overcoat, a slight loss of sensitivity and a change in Photo-induced Discharge Characteristics (PIDC) shape may develop resulting from very low hole mobilities in the overcoat layer. When less than about 3 percent by weight of hydroxy functionalized aromatic diamine and hydroxy functionalized triarylamine is present in the overcoat, charge transport is small resulting in a high residual potential observed across the overcoat. The overcoating of this invention is hole transporting. If the amount of hydroxy functionalized aromatic diamine and hydroxy functionalized triary-

lamine in the overcoat exceeds about 60 percent by weight based on the total weight of the dried overcoating layer, crystallization may occur resulting in residual cycle-up. If the amount of hydroxy functionalized aromatic diamine and hydroxy functionalized triarylamine in the overcoat exceeds about 75 percent by weight based on the total weight of the dried overcoating layer, crystallization occurs resulting in residual cycle-up as well as high wear when operated under bias charging roll conditions. In addition, mechanical properties, abrasive wear, and the adhesion properties may be impacted. Satisfactory results may be achieved when the ratio of hydroxy functionalized triarylamine to hydroxy functionalized aromatic diamine is between about 0.1 to about 2. Preferably, the ratio of hydroxy functionalized triarylamine to hydroxy functionalized aromatic diamine is between about 0.2 to about 1. Too little hydroxy functionalized triarylamine results in a composition that is prone to corona deletion and too high a concentration of hydroxy functionalized triarylamine results in a reduction in wear life (or increased wear rates). Although not intended to be limited by theory, it is hypothesized that hydrogen bonding might occur between the amide ( $-\text{CONR}_2$ ) groups of the polyamide and the hydroxy groups ( $-\text{OH}$ ) of the hydroxy functionalized triarylamine and hydroxy functionalized aromatic diamine during formation of the overcoating layer.

The thickness of the continuous overcoat layer selected depends upon the abrasiveness of the charging (e.g., bias charging roll), cleaning (e.g., blade or web), development (e.g., brush), transfer (e.g., bias transfer roll), etc., system employed and can range up to about 10 micrometers. A thickness of between about 1 micrometer and about 5 micrometers in thickness is preferred. Any suitable and conventional technique may be utilized to mix and thereafter apply the overcoat layer coating mixture to the charge generating layer. Typical application techniques include spraying, dip coating, roll coating, wire wound rod coating, and the like. Drying of the deposited coating may be effected by any suitable conventional technique such as oven drying, infrared radiation drying, air drying and the like. The dried overcoating of this invention should transport holes during imaging and should not have too high a free carrier concentration. Free carrier concentration in the overcoat increases the dark decay. Preferably the dark decay of the overcoated layer should be the same as that of the unovercoated device.

Prolonged attempts to extract the highly fluorescent hydroxy functionalized aromatic diamine hole transport molecule from the crosslinked overcoat, using long exposure to branched hydrocarbon solvents, revealed that the transport molecule is completely immobilized. Thus, when UV light is used to examine the hydrocarbon extract or the applicator pad, no fluorescence is observed. The molecule, in addition to being trapped in the web, is also held in the overcoat by hydrogen bonding to amide groups on the acrylated polyamide. Therefore, the crosslinked overcoat of this invention is substantially insoluble in any solvent in which it was soluble prior to crosslinking and insoluble in and non-absorbing in liquid ink vehicles.

Although it is not entirely clear, some interaction, e.g. hydrogen bonding, may or may not occur between the components combined to form the overcoating layer. Thus, the final overcoating layer of the photoreceptor of this invention includes the recited components in the overcoating layer in non-interacted form, hydrogen bonded form or any other interacted form which inherently occurs when the recited components are combined to form the overcoating layer.

Other suitable layers may also be used such as a conventional electrically conductive ground strip along one edge of the belt or drum in contact with the conductive surface of the substrate to facilitate connection of the electrically conductive layer of the photoreceptor to ground or to an electrical bias. Ground strips are well known and usually comprise conductive particles dispersed in a film forming binder.

In some cases an anti-curl back coating may be applied to the side opposite the photoreceptor to provide flatness and/or abrasion resistance for belt or web type photoreceptors. These anti-curl back coating layers are well known in the art and may comprise thermoplastic organic polymers or inorganic polymers that are electrically insulating or slightly semiconducting.

The photoreceptor of this invention may be used in any conventional electrophotographic imaging system such as copiers, duplicators, printers, facsimile and multifunctional systems. As described above, electrophotographic imaging usually involves depositing a uniform electrostatic charge on the photoreceptor, exposing the photoreceptor to a light image pattern to form an electrostatic latent image on the photoreceptor, developing the electrostatic latent image with electrostatically attractive marking particles to form a visible toner image, transferring the toner image to a receiving member and repeating the depositing, exposing, developing and transferring steps at least once.

A number of examples are set forth herein below and are illustrative of different compositions and conditions that can be utilized in practicing the invention. All proportions are by weight unless otherwise indicated. It will be apparent, however, that the invention can be practiced with many types of compositions and can have many different uses in accordance with the disclosure above and as pointed out hereinafter.

## EXAMPLE I

### Synthesis of Acrylated Elvamide (Structure 1)

To a one-liter, 3-neck, round bottom flask, which was equipped with two stoppers and a mechanical stirrer with a water-cooled bearing, and situated in an oil bath, was added Elvamide 8063 (17.85 grams), acrylic acid (500 grams), and paraformaldehyde (14.28 grams). The mixture was heated at 150° F. for 4 hours. A solution had formed within the first 1.5 hours of heating. The solution was added to water (2 gallons) to precipitate a white, tacky polymer using a Waring blender. The polymer was collected and washed with 2 more gallons of water. The polymer in methanol was filtered and then reprecipitated into water. Ethanol was added to dissolve the polymer. The resultant solution was filtered and then concentrated using a rotary evaporator to yield 69.57 grams of a 15 weight percent resin solids solution in ethanol, as determined by the loss on drying at 125° C. of a 3 gram sample of the solution. The resulting acryoxymethyl modified polyamide can be represented by the following structure:



Acryloxymethyl-Elvamide (Structure 1)

10

**Acryloxymethyl-Elvamide (Structure 1)**  
 A polymer solution in ethanol (31.08 grams) at 12.85 weight percent resin solids in ethanol was formulated with 2 grams of N-(3-hydroxyphenyl)-N-bis(4-methylphenyl)amine (DTAP), 2 grams of N,N'-diphenyl-N,N'-bis(3-hydroxyphenyl)-[1,1'-biphenyl]-4,4'-diamine (DHTBD), and 0.3 grams of azobisisobutyronitrile (AIBN). Successive dilutions were carried out to obtain 11, 10, and 9 weight percent resin solids solutions. The 9 weight percent resin solids solution was determined to be the optimum for the Tsukiage coating of overcoats onto organic photoconductive drums. Tsukiage apparatus is an apparatus employing a ring containing the material through which the drum is inserted. The overcoat thickness was about 5 micrometers after cross linking and drying.

15

20

25

**EXAMPLE II****Synthesis of Acrylated Elvamide (Structure 2)**

To a 500-milliliter, 3-neck, round bottom flask (equipped with two stoppers, a mechanical stirrer with a water-cooled



Acryloxyethoxy-Elvamide (Structure 2)

bearing, and situated in an oil bath) was added Elvamide 8063 (1.0 grams), acrylic acid (211.8 grams), 2-hydroxyethylacrylate (72.5 grams) and paraformaldehyde (8 grams). The reaction mixture was heated at  $150 \pm 10^\circ$  F. for 45 minutes. Stirring was continued and the flask remained in the oil bath until the reaction had returned to  $25^\circ$  C. (which required about 2 hours). The reaction solution was filtered and then was added to water (2 gallons) to precipitate a white, tacky polymer using a Waring blender. The polymer was collected and washed with 2 more gallons of water. The polymer dissolved in ethanol was filtered and then reprecipitated into water. Ethanol was added to redissolve the polymer and the resultant solution was filtered and then concentrated to yield 85.56 grams of a 10 weight percent resin solids solution in ethanol as determined by the loss on drying at  $125^\circ$  C. of a 3 gram sample of the solution. This solution (50 grams at 10 weight percent resin solids) was formulated with DHTBD (2.5 grams), DTAP (2.5 grams), and AIBN (0.3 grams) and then used for the Tsukiage coating of overcoats onto OPC drums as described in Example I.

**Example III**

Two photoreceptors were prepared by forming coatings 50 using conventional techniques on a substrate comprising vacuum deposited titanium layer on a polyethylene terephthalate film. The first coating was a siloxane barrier layer formed from hydrolyzed gamma-aminopropyltriethoxysilane having a thickness of 0.005 micrometer (50 Angstroms). The barrier layer coating composition was prepared by mixing 3-aminopropyltriethoxysilane (available from PCR Research Center Chemicals of Florida) with ethanol in a 1:50 volume ratio. The coating composition was applied by 55 a multiple clearance film applicator to form a coating having a wet thickness of 0.5 mil. The coating was then allowed to dry for 5 minutes at room temperature, followed by curing for 10 minutes at 110 degree Centigrade in a forced air oven. The second coating was an adhesive layer of polyester resin 60 (49,000, available from E.I. duPont de Nemours & Co.) having a thickness of 0.005 micron (50 Angstroms). The second coating composition was applied using a 0.5 mil bar 65

and the resulting coating was cured in a forced air oven for 10 minutes. The next coating was a charge generator layer coated from a solution containing 0.8 gram of trigonal selenium having a particle size of about 0.05 micrometer to 0.2 micrometer and about 0.8 gram poly(N-vinyl carbazole) in about 7 milliliters of tetrahydrofuran and about 7 milliliters of toluene. The generator layer coating was applied with a 0.005 inch Bird applicator and the layer was dried at about 135° C. in a forced air oven to form a layer having a 1.6 micrometer thickness. The transport layer consisted of 50 weight percent N,N'-diphenyl-N,N'-bis(3-methyl-phenyl)-(1,1'-biphenyl)-4,4'-diamine (TPD) dispersed in a 50 weight percent polycarbonate resin [poly(4,4'-isopropylidene-diphenylene carbonate) (available as Makrolon® from Farbenfabriken Bayer A.G.) applied as a solution in methylene chloride solvent. The coated devices were heated in an oven maintained at 80° C. to form a charge transport layer having a thickness of 25 micrometers. The acrylated polyamide (Structure 1)-AIBN formulation (without oxalic acid) was coated on one of the layered devices. The overcoat layer was coated using a 1 mil Bird applicator bar, air-dried, and then oven cured at 120° C. for 30 minutes. Electrical scanner data for this sample are summarized in Table 1. Vo is the initial potential after the charging step. The initial slope of the photo-induced discharge curve (PIDC) is termed S and the residual potential after the erase step is termed Vr. Vdark decay, 1 sec is the dark decay during one second after the charging step. The residual cycle-up voltage after 10,000 cycles of charge, expose, and erase steps is shown. The Vr value is higher for the overcoated sample but is within a usable range. The overcoat had no deleterious effects on the functional electrical properties of the photoreceptor.

TABLE 1

[PIDC Electrical Data For Acryloxyethyl-Elvamide (Structure 1) On Layered Device Containing Trigonal Selenium Particles In Generator Layer And Makrolon/TPD in Transport Layer]

| Sample                                     | Overcoat thickness | Vo  | Vdark decay, (1 sec) | S     | Vr   | V cycle-up (10 Kc) |
|--------------------------------------------|--------------------|-----|----------------------|-------|------|--------------------|
| Acryloxy-methyl-Elvamide/ DHTBD/ PTAP/AIBN | 4.87 +/- 0.8       | 800 | 271.4                | 335.5 | 74.8 | 6.4                |
| Control Trig Se layered device             | No overcoat        | 799 | 260.5                | 274.7 | 15.2 | 2.6                |

There was no appreciable bias charging roll wear of the overcoated device after 100,000 cycles using a bias charging roll-bias transfer roll wear-test fixture.

#### EXAMPLE IV

Two photoreceptors were prepared by forming coatings using conventional techniques on a substrate comprising vacuum deposited titanium layer on a polyethylene terephthalate film. The first coating was a siloxane barrier layer formed from hydrolyzed gamma-aminopropyltriethoxysilane having a thickness of 0.005 micrometer (50 Angstroms). The barrier layer coating composition was prepared by mixing 3-aminopropyltriethoxysilane (available from PCR Research Center Chemicals of Florida) with ethanol in a 1:50 volume ratio. The coating composition was applied by a multiple clearance film applicator to form a coating having a wet thickness of 0.5 mil. The coating was then allowed to

dry for 5 minutes at room temperature, followed by curing for 10 minutes at 110 degrees Centigrade in a forced air oven. The second coating was an adhesive layer of polyester resin (49,000, available from E.I. duPont de Nemours & Co.) having a thickness of 0.005 micron (50 Angstroms). The second coating composition was applied using a 0.5 mil bar and the resulting coating was cured in a forced air oven for 10 minutes. This adhesive interface layer was thereafter coated with a photogenerating layer containing 40 percent by volume hydroxygallium phthalocyanine and 60 percent by volume of a block copolymer of styrene (82 percent)/4-vinyl pyridine (18 percent) having a Mw of 11,000. This photogenerating coating composition was prepared by dissolving 1.5 grams of the block copolymer of styrene/4-vinyl pyridine in 42 mL of toluene. To this solution was added 1.33 grams of hydroxygallium phthalocyanine and 300 grams of 1/8 inch diameter stainless steel shot. This mixture was then placed on a ball mill for 20 hours. The resulting slurry was thereafter applied to the adhesive interface with a Bird applicator to form a layer having a wet thickness of 0.25 mil. This layer was dried at 135° C. for 5 minutes in a forced air oven to form a photogenerating layer having a dry thickness 0.4 micrometer. The next applied layer was a transport layer which was formed by using a Bird coating applicator to apply a solution containing one gram of N,N'-diphenyl-N,N'-bis(3-methyl-phenyl)-(1,1'-biphenyl)-4,4'-diamine (TPD) and one gram of polycarbonate resin poly(4,4'-isopropylidene-diphenylene carbonate) (available as Makrolon® from Farbenfabriken Bayer A.G.) dissolved in 11.5 grams of methylene chloride solvent. The N,N'-diphenyl-N,N'-bis(3-methyl-phenyl)-(1,1'-biphenyl)-4,4'-diamine (TPD) is an electrically active aromatic diamine charge transport small molecule whereas the polycarbonate resin is an electrically inactive film forming binder. Each coated device was dried at 80° C. for half an hour in a forced air oven to form a dry 25 micrometer thick charge transport layer.

#### EXAMPLE V

40 A device was prepared by overcoating a photoreceptor of Example IV with an overcoat layer material of this invention. The overcoat layer was prepared with the following formulation: acrylated Elvamide (1 part by weight), N,N'-diphenyl-N,N'-bis(3-hydroxyphenyl)-[1,1-biphenyl]-4,4'-diamine (a hydroxy functionalized aromatic diamine also called DHTBD, 1 part by weight) and N-(3-hydroxyphenyl)-N-(4-methylphenyl)-N-phenyl amine (a hydroxy functionalized triarylamine, DTAP, 1 part by weight) and azobisisobutyronitrile (AIBN, 0.05 part by weight) in ethanol at 9 weight percent resin solids and roll milled for 2 hours. An overcoat approximately 4 micrometers thick was coated with a one mil Bird bar. This overcoat layer was air dried in a hood for 30 minutes. The air dried film was then dried in a forced air oven at 120° C. for 30 minutes. The adhesion of the overcoat to the charge transport layer was determined to be greater than 16 grams per cm which is high enough to prevent delamination. The overcoat was resistant to rubbing with a methanol swab indicative that crosslinking had taken place without acids.

#### EXAMPLE VI

Devices of Example IV (device without the overcoat), Example V (device with the cross linked overcoat of this invention) were first tested for xerographic sensitivity and cyclic stability. Each photoreceptor device was mounted on a cylindrical aluminum drum substrate which was rotated on

a shaft of a scanner. Each photoreceptor was charged by a corotron mounted along the periphery of the drum. The surface potential was measured as a function of time by capacitively coupled voltage probes placed at different locations around the shaft. The probes were calibrated by applying known potentials to the drum substrate. The photoreceptors on the drums were exposed by a light source located at a position near the drum downstream from the corotron. As the drum was rotated, the initial (pre-exposure) charging potential was measured by voltage probe 1. Further rotation led to the exposure station, where the photoreceptor was exposed to monochromatic radiation of known intensity. The photoreceptor was erased by a light source located at a position upstream of charging. The measurements made included charging of the photoreceptor in a constant current or voltage mode. The photoreceptor was charged to a negative polarity corona. As the drum was rotated, the initial charging potential was measured by voltage probe 1. Further rotation lead to the exposure station, where the photoreceptor was exposed to monochromatic radiation of known intensity. The surface potential after exposure was measured by voltage probes 2 and 3. The photoreceptor was finally exposed to an erase lamp of appropriate intensity and any residual potential was measured by voltage probe 4. The process was repeated with the magnitude of the exposure automatically changed during the next cycle. The photodischarge characteristics was obtained by plotting the potentials at voltage probes 2 and 3 as a function of light exposure. The charge acceptance and dark decay were also measured in the scanner. A slight increase in sensitivity was observed in the overcoated photoreceptors. This increase corresponded to the three micrometer increase in thickness due to the presence of the overcoatings. The residual potential was equivalent (15 volts) for both photoreceptors and no cycle-up was observed when cycled for 10,000 cycles in a continuous mode. The overcoat clearly did not introduce any deficiencies.

#### EXAMPLE VII

##### Deletion Resistance Test

A negative corotron was operated (with high voltage connected to the corotron wire) opposite a grounded electrode for several hours. The high voltage was turned off, and the corotron was placed (or parked) for thirty minutes on a segment of the photoconductor device being tested. Only a short middle segment of the photoconductor device was thus exposed to the corotron effluents. Unexposed regions on either side of the exposed regions were used as controls. The photoconductor device was then tested in a scanner for positive charging properties for systems employing donor type molecules. These systems were operated with negative polarity corotron in the latent image formation step. An electrically conductive surface region (excess hole concentration) appears as a loss of positive charge acceptance or increased dark decay in the exposed regions (compared to the unexposed control areas on either side of the short middle segment). Since the electrically conductive region is located on the surface of the photoreceptor device, a negative charge acceptance scan is not affected by the corotron effluent exposure (negative charges do not move through a charge transport layer made up of donor molecules). However, the excess carriers on the surface cause surface conductivity resulted in loss of image resolution and, in severe cases, cause deletions. The photoreceptor devices Example IV (without the overcoat) and of Example V (with overcoat of the present invention) were tested for deletion

resistance. The region not exposed to corona effluents charged to 1000 volts positive in both cases. However, the corona exposed region of device of Example IV charged to 550 volts (a loss of 450 volts of charge acceptance) whereas the corona exposed region of Example V device charged to 875 volts (a loss of only 125 volts of charge acceptance). The overcoat of this invention has improved deletion resistance by a factor of approximately 4.

#### EXAMPLE VIII

Four electrophotographic imaging members were prepared by applying by dip coating a charge blocking layer onto the rough surface of eight aluminum drums having a diameter of 4 cm and a length of 31 cm. The blocking layer coating mixture was a solution of 8 weight percent polyamide (Nylon 6) dissolved in 92 weight percent butanol, methanol and water solvent mixture. The butanol, methanol and water mixture percentages were 55, 36 and 9 percent by weight, respectively. The coating was applied at a coating bath withdrawal rate of 300 mm/minute. After drying in a forced air oven, the blocking layers had thicknesses of 1.5 micrometers. The dried blocking layers were coated with a charge generating layer containing 2.5 weight percent hydroxy gallium phthalocyanine pigment particles, 2.5 weight percent polyvinylbutyral film forming polymer and 95 weight percent cyclohexanone solvent. The coatings were applied at a coating bath withdrawal rate of 300 millimeters/minute. After drying in a forced air oven, the charge generating layers had thicknesses of 0.2 micrometers. The drums were subsequently coated with charge transport layers containing N,N'-diphenyl-N,N'-bis(3-methylphenyl)-1,1'-biphenyl-4,4'-diamine (TPD) dispersed in polycarbonate (PCZ200, available from the Mitsubishi Chemical Company). The coating mixture consisted of 8 weight percent N,N'-diphenyl-N,N'-bis(3-methylphenyl)-1,1'-biphenyl-4,4'-diamine, 12 weight percent binder and 80 weight percent monochlorobenzene solvent. The coatings were made in a Tsukiage dip coating apparatus. After drying in a forced air oven for 45 minutes at 118° C., the transport layers had thicknesses of 20 micrometers.

#### EXAMPLE IX

Two of the drums of Example VIII were overcoated with an overcoat layer containing a mixture of N,N'-diphenyl-N,N'-bis(3-hydroxyphenyl)-[1,1'-biphenyl]-4,4'-diamine (a hydroxy functionalized aromatic diamine) and N-(3-hydroxy phenyl)-N-(4-methyl phenyl)-N-phenyl amine (a hydroxy functionalized triarylamine) and acryloxyethyl Elvamide and a catalyst AIBN. The overcoat solution was prepared as described in Example V. Approximately 4 micrometer thick overcoats were applied in the dip coating apparatus with a pull rate of 190 mm/min. The overcoated drums were dried at 120° C. for 30 minutes.

#### EXAMPLE X

The electrical properties of the photoconductive imaging samples prepared according to Examples VII and VIII were evaluated with a xerographic testing scanner. The drums were rotated at a constant surface speed of 5.66 cm per second. A direct current wire scorotron, narrow wavelength band exposure light, erase light, and four electrometer probes were mounted around the periphery of the mounted photoreceptor samples. The sample charging time was 177 milliseconds. The exposure light had an output wavelength

of 775 to 785 nm and the erase light had an output wavelength of 680 to 720 nm. The relative locations of the probes and lights are indicated in Table 2 below:

TABLE 2

| Element | Angle (Degrees) | Position | Distance From Photoreceptor |
|---------|-----------------|----------|-----------------------------|
| Charge  | 0               | 0        | Screen at 2 mm              |
| Probe 1 | 26              | 9.1 mm   |                             |
| Expose  | 45              | 15.7     | N.A.                        |
| Probe 2 | 68              | 23.7     |                             |
| Probe 3 | 133             | 46.4     |                             |
| Erase   | 288             | 100.5    | N.A.                        |
| Probe 5 | 330             | 115.2    |                             |

The test samples were first rested in the dark for at least 60 minutes to ensure achievement of equilibrium with the testing conditions at 50 percent relative humidity and 72° F. Each sample was then negatively charged in the dark to a potential of about 385 volts. The charge acceptance of each sample and its residual potential after discharge by front erase exposure to 400 ergs/cm<sup>2</sup> were recorded. The test procedure was repeated to determine the photo induced discharge characteristics (PIDC) of each sample by different light energies of up to 40 ergs/cm<sup>2</sup>. A slight increase in sensitivity was observed in the overcoated devices. This increase corresponded to the approximately 4 micrometer increase in thickness due to the overcoating. The residual potential was equivalent (15 volts) for both devices and no cycle-up was observed when cycled for 100 cycles in a continuous mode. The overcoat clearly did not introduce any electrical deficiencies.

## EXAMPLE XI

The photoreceptors of Example VIII and IX were print tested in a Xerox 4510 machine for 500 consecutive prints. There was no loss of image sharpness, no problem with background or any other defect resulting from the overcoats.

## EXAMPLE XII

The photoreceptors of Examples VIII and IX were tested in a wear fixture that contained a bias charging roll for charging. Wear was calculated in terms of nanometers/kilocycles of rotation (nm/Kc). Reproducibility of calibration standards about  $\pm 2$  nm/Kc. The wear of the drum without the overcoat of Example VIII was  $>80$  nm/kcycles. Wear of the overcoated drums of the current invention of Example IX was  $\sim 40$  nm/kcycles. Thus, the improvement in resistance to wear for the photoreceptor of this invention, when subjected to bias charging roll conditions, was very significant.

## EXAMPLE XIII

Photoreceptors of Examples VIII and IX were contacted with gauze pads soaked with Isopar M, a C<sub>15</sub> branched hydrocarbon (available from Exxon Chemical Inc) useful in liquid ink development xerography. When the pad which contacted the unovercoated photoreceptor Example VIII was exposed to an ultraviolet lamp, telltale fluorescence (characteristic of the transport molecule) was observed on the pad whereas the pad which contacted the crosslinked overcoating of the photoreceptors of Example IX showed no evidence of fluorescence, indicating that the crosslinked sample was resistant to Isopar extraction.

Although the invention has been described with reference to specific preferred embodiments, it is not intended to be

limited thereto, rather those having ordinary skill in the art will recognize that variations and modifications may be made therein which are within the spirit of the invention and within the scope of the claims.

What is claimed is:

1. A crosslinkable coating composition comprising an alcohol soluble acrylated polyamide containing alkoxyethyl or alkoxyalkylmethyl groups attached to amide nitrogen atoms, a crosslinking catalyst and a mixture of a hydroxy functionalized aromatic diamine with a hydroxy functionalized triarylamine.

2. A crosslinkable coating composition according to claim 1 wherein the acrylated polyamide is selected from the group consisting of materials represented by formulae selected from the group consisting of I and II below:

I



wherein:

n is a positive integer sufficient to achieve a weight average molecular weight between about 5000 and about 100,000,

R is an alkylene group containing 1 to 10 carbon atoms, between 1 and 99 percent of the R<sub>2</sub> sites are



wherein

X is selected from the group consisting of —H (acrylate), —CH<sub>3</sub> (methacrylate), alkyl and aryl, and the remainder of the R<sub>2</sub> sites are selected from the group consisting of —H, —CH<sub>2</sub>OCH<sub>3</sub>, and —CH<sub>2</sub>OH, and

II



wherein:

m is a positive integer sufficient to achieve a weight average molecular weight between about 5000 and about 100,000,

R and R<sub>1</sub> are independently selected from an alkylene group containing 1 to 10 carbon atoms, between 1 and 99 percent of R<sub>3</sub> and R<sub>4</sub> are independently selected from the group consisting of

31



or H, methyl, alkyl, aryl, alkylaryl,  $\text{CH}_2\text{OCH}_3$ , and/or  $\text{CH}_2\text{OH}$

wherein

X is selected from the group consisting of —H, alkyl, aryl and alkylaryl, wherein the alkyl groups contain 1 to 10 carbon atoms and the alkylaryl groups contains 1 to 3 alkyl groups,

y is an integer between 1 and 10 and

the remainder of the  $\text{R}_3$  and  $\text{R}_4$  groups are selected from the group consisting of —H, — $\text{CH}_2\text{OH}$ , — $\text{CH}_2\text{OCH}_3$ , and — $\text{CH}_2\text{OCC(O)}-\text{C}(X)=\text{CH}_2$ .

3. A crosslinkable coating composition according to claim 1 wherein the hydroxy functionalized aromatic diamine is represented by the following formula:



wherein

Z is selected from the group consisting of:



n is 0 or 1,

Ar is selected from the group consisting of:



R is selected from the group consisting of — $\text{CH}_3$ , — $\text{C}_2\text{H}_5$ , — $\text{C}_3\text{H}_7$ , and — $\text{C}_4\text{H}_9$ ,

Ar' is selected from the group consisting of:



32

X is selected from the group consisting of:



s is 0, 1 or 2, the hydroxy functionalized aromatic diamine compound being free of any direct conjugation between the —OH groups and the nearest nitrogen atom through one or more aromatic rings.

4. A crosslinkable coating composition according to claim 1 wherein the hydroxy functionalized triarylamine is represented by the following formula:



wherein

Ar is selected from the group consisting of:



R is selected from the group consisting of — $\text{CH}_3$ , — $\text{C}_2\text{H}_5$ , — $\text{C}_3\text{H}_7$  and — $\text{C}_4\text{H}_9$ , Ar' and Ar'' being independently selected from the group consisting of



R is selected from the group consisting of — $\text{CH}_3$ , — $\text{C}_2\text{H}_5$ , — $\text{C}_3\text{H}_7$  and — $\text{C}_4\text{H}_9$ , the hydroxy functionalized triarylamine compound being free of any direct conjugation between the —OH groups and the nearest nitrogen atom through one or more aromatic rings.

5. A crosslinkable coating composition according to claim 1 wherein the composition also comprises free radical initiators to accelerate thermal crosslinking.

6. A crosslinkable coating composition according to claim 5 where the free radical initiator is azobisisobutyronitrile.

7. A crosslinkable coating composition according to claim 1 wherein the composition also comprises a photochemical cure initiator to promote crosslinking.

8. A crosslinkable coating composition according to claim 7 wherein the photochemical cure initiator is Michler's ketone.

9. A method of forming a coating comprising providing a substrate, forming a coating of a crosslinkable composition on said substrate, the crosslinkable coating composition

**33**

comprising an acrylated polyamide containing acryloxymethyl or acryloxyalkylmethyl groups attached to amide nitrogen atoms and a mixture of a hydroxy functionalized aromatic diamine with a hydroxy functionalized triarylamine, and crosslinking the acrylated polyamide.

**10.** A method of forming a coating according to claim **9** comprising crosslinking the polyamide with heat.

**11.** A method of forming a coating according to claim **10** comprising crosslinking the polyamide with heat in the presence of a free radical initiator.

**34**

**12.** A method of forming a coating according to claim **11** wherein the free radical initiator is azobisisobutyronitrile.

**13.** A method of forming a coating according to claim **9** comprising photochemically crosslinking the polyamide in the presence of a photochemical initiator.

**14.** A method of forming a coating according to claim **13** wherein the photochemical initiator is Michler's ketone.

\* \* \* \* \*